# EUROPEAN PATENT APPLICATION

(11) **EP 0 159 457 A1**
(43) Date of publication of application: **30.10.1985**
(21) Application number: 84830130.5
(22) Date of filing: 26.04.1984
(51) Int. Cl.: B27N 5/00, B27N 1/02

(54) **molded furniture panels method production and furniture panels relative**

(71) Applicant: SOL.MAR. DI SOLDERA FIORENZO E MARTINUZZO ALBERTO s.a.s., I-31040 Mansue' (Treviso) (IT)
(72) Inventor: Martinuzzo, Alberto, I-31040 Gorgo al Monticano (Treviso) (IT)
(74) Representative: D'Agostini, Giovanni, Dr.

(57) **Abstract**

A method for carrying out furniture door panels of variable thickness, the preferred thickness being 5 to 35 mm, characterised in that it comprises:
- using as raw material wood saw dust, even from sawmill or wood-working waste, provided it is of sufficiently fine grain;
- mixing said wood saw dust with a polyurethan product (1) of the high density rigid polymerization type, that is with minimum generation of gas;
- hot pressing rapidly the mixture thus obtained between heated die and counterdie, at least one of which with molded surface, with eventual prearrangement of a sheet of wood or laminated plastic (2, 3) between the surfaces of said dies and the mixture.

With this method very strong, aesthetically valued and very cheap panels for furniture doors are obtained.

## Description

The present invention relates to a method for producing molded surface panels for furniture and panels and furniture thus obtained.

The invention is particularly useful for carrying out central panels which are successively square framed for producing furniture doors.

At the current state of the art the need is well known of producing door panels molded with drawings or decorations generally in high-relief on an outside face for being then framed in order to form a door of a wooden piece of furniture. These door paiiels are made:
1. or in massive wood,
2. or by strong pressing squares of wooden shaving panels covered with glued sheet of wood for impressing a permanent set mold,
3. or by foaming cellular polyurethane within two sheets of .wood one of which is molded in order to have the desired drawing.

The disadvantages of these currently-used known embodiments consist essentially in that:
- in case 1., wood and manufacturing costs are too high for average productions;
- in case 2., the deformation of a wooden shaving panel can be only of a limited amount so complex drawings cannot be made, and furthermore glueing costs are to be considered;
- in case 3., the molded sheet of wood has to be preformed before effecting foaming of cellular polyurethane between die and counterdie.

The object of the present invention is to obviate the above-mentioned disadvantages and particularly to produce door central panels at a very low cost.

The invention as claimed solves the problem of how to carry out furniture door panels with variable thickness, the preferred range being 5 to 35 mm thickness, by means of the following method:
- using as raw material wood saw dust, even from wood sawmill or wood-working waste provided it has a sufficiently fine grain;
- mixing said wood saw dust with a polyurethane with a low foaming gas developping, of high density and rigid polymerization foaming type;
- hot-pressing rapidly the mixture thus obtained between preferable heated die and counterdie, being at least one of which provided with molded surface, with eventual prearrangement of a sheet of wood or laminated plastic between the surfaces of said dies and the mixture, with pressure ranging between 100 and 350 ton/sq.cm., the preferred range being 150 to 300 ton/sq.cm.

In a preferred embodiment of the invention the method comprises:
- a first mixing of the wood saw dust with bifunctional products such as glicols or organic polyester compounds containing carboxyl group (-COOH) or low gas generation polyols;
- then a second mixing of the wood saw dust mixture obtained by the first mixing with a diisocyanate containing two functional groups of structure (-NCO); and finally .
- rapid transfer to pressing between die and counterdie.

In another preferred embodiment of the invention the method includes:
- a first mixing of the wood saw dust with polyols and carbon naphtha in a ratio of about 10% weight of wood saw dust;
- then a second mixing of the wood saw dust mixture obtained by the first mixing with about 10% weight of diisocyanate; and finally
- rapid transfer to pressing between die and counterdie within one minute from the second mixing.

In a further preferred embodiment of the invention the method comprises:
- using in the first mixing a polyol product mixed with 50% weight of carbon naphtha.

In a further preferred embodiment of the invention the method comprises:
- preparing a polyol product consisting of about 40 wt % of POLIOLO G790 ATLAS EUROPOL and about 60 wt % POLIOLO TF ATLAS EUROPOL, trade names of polyols supplied by Atlas Europol of Ternate Varese, Italy;
- pre-mixing said polyol compound product with CARBON NAPHTHA in approximately equal ratios;
- carrying out said first mixing with said wood saw dust of this pre-mixing,
- carrying out said second mixing with diisocyanate or isocyanate compound i.e. DIISOCIANATO HD ATLAS EUROPOL;
- pressing the product forming the panel as claimed.

In a further embodiment of the invention the method comprises carrying out said first and second mixing of the wood saw dust in the same blender by mixing on vertical axis cylindrical chamber with radial arms rotating at about 1500 r.p.m. speed, by immediately successive inlet first of the polyol-carbon naphtha compound product and then of the diisocyanate product, coming from two separate tanks which disembogue by means of two separate ducts, into said blender.

In a further preferred embodiment of the invention the method comprises effecting said pressing at a temperature of about ⁵0°C.

In a further preferred embodiment of the invention the method comprises carrying out said pressing between die and counterdie wherein the lower plane is movable and supports passing a plurality of thrust lifting vertical pins positioned under a movable matrix die with the upper surface having the shape to be given to the corresponding panel surface, which slides vertically in a matrix guide box open upwards for receiving the punch of the upper counterdie hung fixed on the upper plane, a fixed plane being arranged under said vertical lifting pins so that:
- after eventually placing the covering sheet for the molded surface on the matrix of the lower die and applying thereon the convenient amount of wood saw dust with polyurethane foaming mixture and eventually on this one another covering sheet;
- the lower die is lifted against the upper one until the flat surface upper punch enters the guide box of the lower die determining the pressing;
- the lower die is lowered with the respective support plane and lifting pins until the latter beat against the underlying fixed plane consequentely getting out into the cointaining box of the lower die matrix urging same upwards for extraction.

In a further preferred embodiment of the invention the method comprises carrying out said pressing for about 1 minute if the panel to be obtained is bare, i.e. not covered, or for about 2 minutes if the panel is covered with said sheets.

The advantages offered by this invention are essentially that production costs are extremely low as waste wood saw dust is used and the product if not covered can be lacquered, if covered appears aesthetically finished like massive wood.

One way of carrying out the invention is described in detail below with reference to drawings which illustrate one preferred embodiment, in which:
Figure 1 is an enlarged sectional transversal scrap view of the central panel of the furniture doors, covered with sheet of wood on the opposite surfaces, obtained by the method of the invention; Figure 2 is a diagram of the production system;
Figure 3 is a perspective view of the panel mounted on the frame thereof in order to form a furniture door; Figure 4 is a sectional transversal view of the furniture door of Figure 3.

As shown in the above-mentioned figures, the invention provides the realization of a panel (A) comprising a polymerized mixture of wood saw dust with polyurethane (1) covered above and below with sheets of wood (2,3) the outside surface of which is molded by pressing in a press (D) where polymerization reaction and wood saw dust mixture in one block occur. The covering sheets (2,3) may also lack when the furniture door is to be lacquered. The panel thus obtained (A) is then mounted on a door frame (B) in successive operations which are not related to the present invention.

The production system provides a mixing unit (C) comprising a wood saw dust feeder, such as a screw feeder (5) which supply wood saw dust from a wood saw dust tank (4) and pours same into a hopper (6) provided with motorized (7') mixer-conveyor (7), which causes wood saw dust to flow in dosed amount into a vertical mixing chamber (8) provided with motorized (9') vertical rotating blendor (9). The mixing chamber (8) is provided with various opposite joints at various levels of mixture fluid inlet (10) which engage two respective ducts (11',12') so that the respective mixture fluid products flow in adjustable manner in controlled amount from separate independent tanks (11,12) one containing mixed polyols compounds together with carbon naphtha and the other containing diisocyanate compound. At the base of the mixing chamber (8) an opening for unloading the mixture (13) is provided, with chute (14) which supplies the almost powdery mixture on a belt conveyor (15) which conveys same to the press (D). The press (D) includes a fixed upper plane (22) and a fixed lower plane (17) which supports cylinders (18) which passing rods (18') lift and lower a movable overhanging lower plane (16) provided with passing vertically movable stripper pins (19), the lower die being fixed thereon, consisting of a matrix (20), with molded upper surface for molding the surface of the panel to be pressed (A), vertically guided movable within a guide box (20'), while the upper counterdie (21) is fixed under the upper plane (22). Pressing is carried out during lifting of the movable lower plane (16) and panel (A) extraction occurs during lowering, since the pins (19) beating on the fixed lower plane (17) get out upwards urging the matrix (20) with the pressed panel (A) outside the die guide box (20').

### RESULTS OF TESTS.

A 407x394x15 mm specimen panel obtained by means of the above-mentioned method has been subjected to WET/DRY TEST at "CATAS CENTRO REGIONALE ASSISTENZA TECNICA SETTORE SEDIE MOBILI LEGNO", a Regional Laboratory of the Chamber of Commerce Industry Handicraft and Agriculture of Udine, (IT) in the Laboratory Section of SAN GIOVANNI AL NATISONE (UD), IT. Method: No. 1 cycle comprising: 10 days at 35-40% r.h. at 23°C temperature.

### Results:

a) - weight change with respect to initial stage:
   - wet + 5.6%
   -dry
b) - average thickness change with respect to initial stage:
   -wet + 3.5%
   -dry + 0.7%

c) - deformations: practically absent.

As it can be noticed, the results are fully positive.

Of course changes and modifications can be made without departing from the spirit or scope of the invention as defined in the appended claims.

## Claims

1. Method for producing molded surface panels for furniture doors, characterised in that it comprises:
- using as raw material wood saw dust, even waste wood saw dust and even containing impure matter from wood-working;
- mixing said wood saw dust with a rigid polymerization polyutheraii product preferably of high density type, that is with minimum generation of gas;
- hot pressing rapidly the mixture thus obtained between heated die and counterdie, at least one of which being provided with molded surface, with eventual prearrangement of a sheet of wood or laminated plastic between the surfaces of said dies and the mixture, and keeping under pressing so that its complete foaming be impeded and the mixture be kept pressed until complete hardening with a pressure ranging from 100 to 350 ton/sq.cm., the preferred range being 150 to 300 ton/sq.cm..

2. A method as claimed in claim 1, wherein said method further comprises:
- a first mixing of the wood saw dust with bifunctional products such as glicols or organic polyester compounds containing the carboxyl group (-COOH) or polyols;
- a second mixing of the wood saw dust mixture obtained by the first mixing with a diisocyanate containing two bifunctional groups of structure (-NCO); and finally
- rapid transfer before the reaction begins or at most at the beginning of same, to pressing between die and counterdie.

3. A method as claimed in claims 1 and 2, wherein said method further comprises:
- a first mixing of wood saw dust with polyols and carbon naphtha in about 10% weight ratio of wood saw dust;
- a second mixing of the wood saw dust mixture obtained by the first mixing with about 10 wt % diisocyanate; and finally
- rapid transfer to pressing between die and counterdie within one minute from the second mixing.

4. A method as claimed in the preceding claims, wherein said method further comprises:
- using in the first mixing a polyol product mixed with carbon naphtha in 50% weight ratio.

5. A method as claimed in the preceding claims, wherein said method further comprises:
- preparing a polyol product consisting of about 40 wt % POLIOLO G790 ATLAS EUROPOL and about 60 wt % POLIOLO TF ATLAS EUROPOL, trade names of polyols supplied by Atlas Europol of Ternate Varese, IT;
- premixing said polyol compound product with CARBON NAPHTHA in approximately equal ratios;
- carrying out said first mixing with said wood saw dust of said premixing;
- carrying out said second mixing with isocyanate compond i.e. DIISOCIANATO HD ATLAS EUROPOL of Ternate IT;
- pressing said product in order to form the panel as claimed.

6. A method as claimed in the preceding claims, characterised in that it further comprises effecting said first and second mixing of wood saw dust in the same blendor by mixing on vertical cylindrical chamber with vertical axis provided with radial rotating arms at about 1500 r.p.m. speed, by letting in successively first the polyol-carbon naphtha compound product and then the diisocyanate product, coming from two separate tanks which penetrate said blendor with two separate ducts.

7. A method as claimed in the preceding claims, characterised in that it further comprises effecting said pressing at a temperature of about 50°C.

8. A method as claimed in the preceding claims, characterised in that it further comprises effecting said pressing between die and counterdie in which the lower plane is movable and supports passing a plurality of thrust lifting vertical pins positioned under a movable matrix with the upper surface having the shape to be given to the corresponding panel surface, said matrix sliding vertically in a matrix guide box open upwards for receiving the punch of the upper counterdie hung up fixed to the upper plane, being a fixed plane placed under said lifting vertical pins so that:
- after eventually placing the covering sheet for the molded surface on the matrix of the lower die and applying thereon the convenient amount of wood saw dust mixture mixed according to the preceding claims and eventually on this one another covering sheet:
- the lower die is lifted against the upper one until the flat surface upper punch enters the lower die guide box determining pressing;
- the lower die is lowered with the respective support plane and lifting pins until the latter beat against the underlying fixed plane getting out consequentely within the containing box of the lower die matrix urging the pressed panel upwards for lifting.

9. A method as claimed in the preceding claims, characterised in that it further comprises effecting said pressing for about 1 minute if the panel to be obtained is bare, that is not lined, or for about 2 minutes if the panel is lined with said sheets.

10. Door panel carried out according to the method of the preceding claims, characterised in that it is made of a mixture of wood saw dust and polyurethane resin oven-cured between die and counterdie so that its complete foaming be impeded.
